

# UNITED STATES PATENT OFFICE

2,314,614

## METHOD FOR PREPARING FILLING MATERIAL FOR INCENDIARY BOMBS AND FLARES

Ernest F. Fisher, Passaic, N. J.

No Drawing. Application December 11, 1941.  
Serial No. 422,555

1 Claim. (Cl. 44—3)

My invention relates to improvements in the manufacture of filling material for incendiary bombs and flares for military and other industrial uses.

The principal ingredients of my bomb are magnesium particles and paper pulp made from wood fiber or other combustibles.

The manufacture of the filling for an incendiary bomb or flare is preferably as follows:

Magnesium in the form of small particles of approximately 500 microns in size is mixed with wood pulp and water in such a proportion that the particles of magnesium are disseminated throughout the mass.

The well agitated mixture of pulp and magnesium particles is filtered through a continuous suction filter, the pulp impregnated with magnesium particles forming a filter cake in the form of a ribbon. This ribbon is dried and is used in various forms as a filler in the bomb. It can be broken in small pieces or used in rolls.

This material burns with an intense heat. The particles of magnesium are close enough together

in the pulp to prolong combustion without burning too rapidly. The pulp fibres form a porous medium through which the magnesium particles are distributed, the magnesium particles being separated from each other by a slower burning combustible, and the requisite oxygen for combustion.

My incendiary bomb filling requires a relatively small amount of magnesium and large powerful combs of great incendiary power can be manufactured with only a few cents worth of magnesium. This material is safe to handle and to store.

I claim:

15 A method of making filling for incendiary bombs consisting of pulping paper and mixing magnesium dust with said pulp and water; agitating this mixture and filtering said mixture to form a uniformly flat sheet or ribbon and finally 20 drying said sheet or ribbon for use in an incendiary bomb.

ERNEST F. FISHER.